

# United States Patent [19]

Murin et al.

[11] 3,876,428

[45] Apr. 8, 1975

[54] **MULTILAYER SILVER HALIDE MATERIAL  
CONTAINING A WHITE COUPLER**

[76] Inventors: **Borys Murin**, Agfa-Gevaert AG, Werk Perutz, Kistlerhofstrasse 75, 8 Munich 25; **Walter Puschel**, Agfa-Gevaert AG, D-5090 Leverkusen-Bayerwerk; **Hans Glockner**, Agfa-Gevaert AG, Werk Perutz, Kistlerhofstrasse 75, 8 Munich 25, all of Germany

[22] Filed: Mar. 11, 1974

[21] Appl. No.: 449,596

## Related U.S. Application Data

[63] Continuation of Ser. No. 247,291, April 25, 1972, abandoned, which is a continuation-in-part of Ser. No. 13,805, Feb. 24, 1970, abandoned.

## Foreign Application Priority Data

Feb. 24, 1969 Germany..... 1909067

[52] U.S. Cl..... 96/74; 96/100

[51] Int. Cl..... G03c 1/40

[58] Field of Search..... 96/100, 74

## References Cited

### UNITED STATES PATENTS

2,998,314 8/1961 Puschel..... 96/100  
3,028,238 4/1962 Puschel et al..... 96/100

3,155,510 11/1964 Nogradi et al..... 96/100  
3,580,722 5/1971 Sakamoto et al..... 96/100

## FOREIGN PATENTS OR APPLICATIONS

914,145 12/1962 United Kingdom..... 96/100

Primary Examiner—J. Travis Brown  
Attorney, Agent, or Firm—Connolly and Hutz

## [57] ABSTRACT

Color photographic material containing as a white coupler of a pyrazolone derivative of the formula



wherein

$\text{R}_1$  is alkyl, substituted or unsubstituted;  
 $\text{R}_2$  is a radical with at least 8 carbon atoms, a phenyl group substituted with sulfo or an  $\text{OR}_4$  group;  
 $\text{R}_3$  is hydrogen or alkyl, halogen, sulfo-group, alkylsulfonyl,

and wherein  $\text{R}_2$  and/or  $\text{R}_3$  may carry a straight or branched aliphatic hydrocarbon radical which prevents diffusion.  $\text{R}_4$  represents a phenyl or a 2-phenoxyethyl group.

**2 Claims, No Drawings**

## MULTILAYER SILVER HALIDE MATERIAL CONTAINING A WHITE COUPLER

This application is a continuation under Rule 60 of copending application Ser. No. 247,291, filed Apr. 25, 1972 by Murin et al. for White Coupler for Multi-Layer Dyestuffs, which application is a continuation-in-part of application Ser. No. 13,805, filed Feb. 24, 1970 both now abandoned.

### BACKGROUND OF THE INVENTION

The invention relates to novel compounds for the improvement of the color quality of multi-layer dye images which are obtained by chromogenic development of imbedded color couplers in color photographic multi-layer materials.

The improvement of the color reproduction of color materials by using the so-called white coupler is known (see W. Pueschel, Mitteilungen aus den Forschungslaboratories [Reports from Research Laboratories] of Agfa-Gevaert AG., Leverkusen-Munich, 1964, Vol. IV, pp. 352-367). The effect of these white couplers is based on the fact that they react with the oxidation products of developer substances to result in colorless compounds. They are used where undesired oxidation products of developer substances should be eliminated in order to avoid a deterioration of the color quality of the image. Generally, a high developing activity is required of such white couplers.

In the German published application No. 1,155,675 and in the British Pat. No. 914,145, there are suggested for the stated purpose inter alia pyrazolone developers carrying in the coupling position an unsubstituted or a substituted alkyl group. The pyrazolone white couplers disclosed in these patents, however, are relatively weak in their developing activity, so that they insufficiently fulfill their purpose of reacting with undesired oxidation products of developer substances. Quickly reacting compounds are therefore of great interest for the preparation of color photographic materials.

It is an object of this invention to provide a color photographic material in which there is reduced secondary color density in the developed material.

It is another object of this invention to provide multi-layer dye containing photographic material having improved characteristics.

A still further object is to minimize color fog and improve the gradation of photographic material by adding pyrazolone white couplers.

10

### SUMMARY OF THE INVENTION

According to the invention, it has been established that the pyrazolone derivatives which are particularly active and consequently are very well suited for the improvement of the color quality of multi-layer dye images, having the following general formula:



wherein  $\text{R}_1$  is a methyl, ethyl or cyanoethyl group;  $\text{R}_2$  is a radical with at least 8 carbon atoms, a phenyl group substituted with sulfo or an  $\text{OR}_4$  group;  $\text{R}_3$  is hydrogen, alkyl, halogen, a sulfo group, alkylsulfonyl;  $\text{R}_4$  represents a phenyl or a 2-phenoxyethyl group; wherein  $\text{R}_2$  and/or  $\text{R}_3$  may carry a diffusion-preventing straight or branched aliphatic hydrocarbon radical.

The acylamino group in the 3-position of the pyrazole ring provides a higher reactivity in the novel white coupler than heretofore obtained. This higher developing activity improves the color quality of the picture.

### DETAILED DESCRIPTION OF THE INVENTION

White couplers of the invention are the following compounds, for example:

40

I.



II.



III<sub>a</sub>



3

1

IV



Compounds II-V are derivatives of carbamic acid. 15 They are particularly suitable for the purpose of the invention. The white couplers of this invention illustrated by Compounds I-VII have in the group in the 3-position of the pyrazole ring the particular group of radicals which provide the improved developing activ- 20 ity.

In the instance where it concerns diffusion-proof compounds, the application of the novel white developers may take place either by imbedding into one or several separating layers between the developer-containing emulsion layers or they may be directly added to the developer-containing emulsion layers. In the first instance, the developing oxidation products

V.



VI.



45 diffusing from an emulsion layer to an adjacent layer are apprehended in the separating layer, whereby a color falsification is avoided. In the second instance, the gradation of a layer may be controlled, which is important for the correct gradation of color shades. In the 50 latter type of application, the advantages of the use of high silver halide amounts may also be utilized.

The novel diffusion-proof white couplers may be introduced into the gelatin separating layer or into the emulsion layer in accordance with known processes. Preferably, dispersions are prepared in a known manner from the water-insoluble compounds. This may take place, for example, by dissolving in a low-boiling solvent, e.g. ethyl acetate, and subsequent dispersion in gelatin solution with the aid of a wetting agent. In order to avoid crystallization of the compounds, a so-called oil former may be employed in addition.

Compounds with sulfo-groups or with carboxyl groups in the form of aqueous-alcoholic solutions of an alkali salt may be added to the gelatin solution or to the emulsion.

65 emulsion.

Non-diffusion proof novel white couplers may also be added to the photographic baths, specifically to the color developer. Used in this manner, color fog can be avoided and the gradation of the material can be controlled.

The diffusing compounds are added to a processing bath in the form of an aqueous, alcoholic or aqueous-alcoholic solution, if necessary with the aid of alkali.

A comparison of the properties of the novel white coupler having the above-mentioned vital group in 3-position with previously known white couplers without an acylamino group in the 3-position of the pyrazole ring, when conducted by dispersing the novel white coupler and the previously known white coupler in identical but separate parts of a gelatin solution containing a blue-green coupler, showed that, on exposure, in the subsequent developed color negative the color density of the blue-green coupler in the part containing the novel white coupler had substantially less density than in the other part. This lesser density is attributable to the higher reactivity of the white coupler of this invention.

The preparation of the novel white couplers may occur according to principally known processes.

#### EXAMPLE I

A color photographic negative material is synthesized as follows:

1. On the carrier a spectral red-sensitized layer which contains a color coupler for blue-green is placed.
2. On that red-sensitized layer is placed a separating layer which contains the white coupler of formula II. The separating layer is ca. 1  $\mu$  thick; the ratio of white coupler to gelatin is 1:2.
3. On that separating layer is placed a green-sensitive layer with a color coupler for purple.
4. A yellow filter layer of colloidal silver.
5. A spectral non-sensitized, hence blue-sensitive, layer with a color coupler for yellow.

As a comparison to this material A, a corresponding material B is synthesized, wherein the separating layer 2 contains no white coupler but only consists of an equally thick gelatin layer.

From assays of both materials are prepared color extract wedges behind the filters blue, green and red. The wedges are then subjected to a normal color negative developing process; color developing substance is N-ethyl-N-(methanesulfonamidoethyl)-3-methyl-4-aminoanilinosulfate.

In comparing the wedges, the following is determined: The purple wedge with white coupler A shows a pure purple, the purple wedge without white coupler B, however, is more bluish tinged. The measurement in the densitometer indicates that the secondary color density behind the red filter in B is about 20% higher than in A. Thus the white coupler of this invention with the described group in the 3-position of the pyrazole ring improves the picture quality in color reproduction of color materials.

The same holds true for both blue-green wedges; The secondary color density behind the green filter without the white coupler is about 15% higher than with the white coupler.

The white coupler employed in this example was prepared as follows:

#### STEP 1

-Methyl-8-imino-8-ethoxy-propionic acid ethyl ester ("methyl-maloniminoether")

To 230 g -cyanopropionic acid ethyl ester in 100 ml absolute alcohol were added 68 g HCl gas while cooling with ice water. Temperature 15°-20°C. The reaction mixture was cooled several days. Then the crystal mass

finely ground with benzine/benzole (1:1) and the crystals separated and washed with benzine/benzole mixture. Dried by means of KOH. Yield 230 g, F. 85°C.

#### STEP 2

p-Methylsulfonyl-hydrazine

276 g p-aminophenyl-methylsulfone in 3 l. water and 520 ml concentrated hydrochloric acid are diazotized with 112 g sodium nitrite in 100 ml water. The diazonium salt solution is poured while stirring into 1680 g Na<sub>2</sub>SO<sub>3</sub>·7H<sub>2</sub>O in 1680 ml water; pH is kept at 7-7.5; heated for one hour to 80°C and then 960 ml concentrated hydrochloric acid are added. Then this was vaporized until dry. The residue was boiled with 1.6 l. water and 0.8 l. concentrated hydrochloric acid for one hour. After cooling drawn off and the precipitate dissolved in 1.5 l. water and then suspended with ammonia to pH 7. After cooling, the precipitated hydrazine is drawn off and dried. Yield 170 g, F. 134°C.

#### STEP 3

1-(4'-Methylsulfo-phenyl)-3-amino-4-methyl-pyrazolone-(5)

25 250 g Methylmaloniminoetherchlorohydrate of step 1 are dissolved in 750 ml methanol and mixed with sodium methylate solution until phenolphthalein remains red. Then it is neutrally suspended with glacial acetic acid (ca. 60 ml.). Thereupon 190 ml hydrazine are 30 added according to step 2 and stirred for one hour. After addition of 1 l. 2n-soda lye it is further stirred for 30 minutes. After filtering 600 ml 2n-hydrochloric acid are added and then suspended with glacial acetic acid to weakly acid. The precipitate is drawn off and washed 35 with warm water. Yield 220-220 g, F. 240°-245°C.

#### STEP 4

2-Tetradecyl-4-chloro-5-methylphenol

40 1,000 g 4-chloro-m-cresol (Raschit) are melted in an oil bath at 70°C and 14 g bor trifluoride are introduced in 10 minutes. In two hours to this are added by drops 393 g 1-tetradecene at 70°C, stirred for one hour, then poured into a mixture of 2 l. water and 0.9 l. soda lye of 30% and well stirred for 5 minutes. After the layers have separated, the aqueous layer is rejected. The oil layer is then washed twice with soda lye, then treated with thinned hydrochloric acid and the oil layer is taken up in 600 ml. methylene chloride. After drying, methylene chloride is evaporated and the residue distilled in vacuo. Yield 520 g, Kp 0.05 mm-165°-170°C.

#### STEP 5

2-(2'-Tetradecyl-4'-chloro-5'-methylphenoxy)-ethanol-(1)

34.5 g sodium are dissolved in 260 ml methanol. In the solution are dissolved now 408 g "phenol" from step 4 while stirring and subsequently 73.5 g 2-chloroethanol are added. After 3 hours again 73.5 g 2-chloroethanol are added and allowed to stand overnight and the next day are boiled for 3 hours in a vapor bath while stirring. The mixture is then poured into 2 l. water and stirred well. The water is removed and the oil layer is dissolved in 600 ml methylene chloride. With the addition of acetic acid it is now washed with water up to the neutral point. After removal of the methylene chloride, there remained 420 g residue. The highly viscous oil is then further processed without purification.

## STEP 6

2-(2'-Tetradecyl-4'-chloro-5'-methylphenoxy)-ethyl-chloroformate-(1)

Into 950 ml toluol (dry) are introduced in 40 minutes while stirring 150 g phosgene. Thereto are added by drops within 3 hours a mixture of 400 g "Phenoxyethanol" from step 5, 126 g dimethylanilin, 100 ml. toluol. After standing overnight there are added to the reaction solution 600 ml cold water and air is blown through until the excess phosgene is removed. The water is separated from the toluol solution, and the toluol solution is additionally thinned with HCl and washed with water. After distilling off the toluol there remain ca. 440 g oily residue with a content of 92-95% of chloroformic acid ester.

## STEP 7

White coupler of the formula



267 g Pyrazolone of Step 3 are dissolved in 1.5 l. pyridine and mixed with 66 g aluminum chloride. The reaction is exothermic. After cooling to 45°C, 490 g chloroformic acid ester of Step 6 (100%) are added and after 40 3 hours poured on thinned hydrochloric acid, the hydrochloric acid then being separated, washed with thinned hydrochloric acid and the oily cake taken up with acetone, treated with animal charcoal and the filtrate mixed with benzine (ca. 4 l.). The acetone is removed by washing with water, the developer being crystallized out, after standing drawn off and washed with benzine. Yield 200-230 g, F. 110°C.

## EXAMPLE II

A highly sensitive color reversal film (film developed by reversal) is synthesized as follows:

1. On the base a spectral red-sensitized emulsion layer rich in silver. The emulsion contains 50 g/kg of the blue-green coupler  $\alpha$ -naphthadicidic octadecylamide. 55 The layer is poured into three variants:

- without white coupler,
  - in addition to the 50 g color coupler 50 g white coupler of Formula III,
  - in addition to the 50 g color coupler 45 g white coupler of Formula III.
  - A gelatin separating layer.
  - A green-sensitive layer with a color coupler for purple.
  - A fadeable yellow filter layer.
  - A spectral unsensitized layer with a color coupler for yellow.
- From the three experimental pourings A, B, and C, color separation wedges are prepared in the customary

manner. The processing of the wedges occurs in a color reversal process. The developing substance is 2-methyl-4-diethylamino-aniline sulfate. The wedges are measured behind red, green and blue filters.

5 The results obtained from behind the red filter characterize the properties of the blue-green layer. The following values are measured, "E<sub>spez</sub>" being the expression for the usable sensitivity and in particular log It of (D<sub>max</sub> + color fog/2)

10

15

|   | D <sub>max</sub> | E <sub>spez</sub> |            |
|---|------------------|-------------------|------------|
| A | 2.78             | 2.14              | Comparison |
| B | 2.18             | 1.87              | + 0.8 DIN  |
| C | 1.60             | 1.30              | + 1.2 DIN  |

The white coupler III mentioned in this Example is prepared as follows:

20

STEP 1  
Color coupler of the formula



was prepared by acylation of 1-(3'-chlorophenyl)-3-aminopyrazolone-(5) with chloroformic acid(m-pentadecylphenyl-ester). Such couplers and the process for their preparation are disclosed in the German published application No. 1,176,479.

STEP 2  
White coupler of the Formula III

21.6 g of the purple coupler of Step 1, 300 ml methanol, 26.5 g acrylonitrile, 1 ml sodium methylate solution (35% in methanol) and 0.2 g hydroquinone dimethyl ether are heated for 5 hours in an autoclave to 120°C. The reaction mixture is concentrated under reduced pressure and the residue is recrystallized from acetic ester petroleum ether. Yield 11.3 g, F. 63°-68°C.

What is claimed is:

1. A multilayer silver halide color photographic material containing a white coupler of the following general formula

5



10

a green-sensitive silver halide emulsion layer containing a color coupler for purple  
a blue sensitive silver halide emulsion layer containing a color coupler for yellow and contained in the photographic material a white coupler of the following formula:



wherein

R<sub>1</sub> represents a methyl, ethyl or cyanoethyl group;  
R<sub>2</sub> represents (1) phenyl substituted with chlorine and/or an alkyl hydrocarbon radical with at least 8 carbon atoms or (2) 2-phenoxyethyl substituted with one or more substituents selected from the group consisting of alkyl and chlorine;

R<sub>3</sub> represents one or several members of the group consisting of hydrogen, halogen, sulfo, thioalkyl and alkylsulfonyl.

2. A silver halide photographic material having multilayer color couplers which comprises the following layers:

a red-sensitive silver halide emulsion layer containing a color coupler for blue-green

15

20

wherein  
R<sub>1</sub> represents a methyl, ethyl or cyanoethyl group;  
R<sub>2</sub> represents (1) phenyl substituted with chlorine and/or an alkyl hydrocarbon radical with at least 8 carbon atoms or (2) 2-phenoxyethyl substituted with one or more substituents selected from the group consisting of alkyl and chlorine;  
R<sub>3</sub> represents one or several members of the group consisting of hydrogen, halogen, sulfo, thioalkyl and alkylsulfonyl.

25

30

\* \* \* \* \*

35

40

45

50

55

60

65